

1

3,788,884  
TEXTILE MATERIAL COATED WITH A  
WATERPROOFING AGENT

André Bernard, Pierre Gagne, and Georges Gras, Villeurbanne, and Jean Neel, Lyon, France, assignors to Societe Civile dite Soltex, Paris, France  
No Drawing. Original application Dec. 16, 1969, Ser. No. 885,620. Divided and this application Feb. 16, 1971, Ser. No. 115,805  
Claims priority, application France, Dec. 19, 1968, 50,775; Nov. 6, 1969, 6938618  
Int. Cl. B44d 1/02

U.S. Cl. 117—121

2 Claims

ABSTRACT OF THE DISCLOSURE

Compounds of the formula



[where R is tolylene or hexamethylene; A and B are  $NHR_1$ ,  $NHR_2$ ,  $N(R_1)_2$ ,  $N(R_2)_2$ ,  $OR_1$ ,  $OR_2$ ,  $R_1$  or  $R_2$ ; and  $R_1$  and  $R_2$  are aliphatic hydrocarbon radicals of 12-22 carbon atoms] are crosslinked on textile fabrics with isocyanates to provide effective and long lasting waterproofing of the fabric.

The present application is a divisional application of U.S. Ser. No. 885,620, filed Dec. 16, 1969.

The present invention relates to new agents for making textiles water-repellent. It also relates to a process of applying these agents to textiles.

Many products are known for waterproofing textiles, e.g. paraffinic waxes; aluminium soaps; complex compounds of chromium; N-methylolamides of fatty acids; pyridinium salts; condensation products of melamine-formol, ureas and formol, and phenol-formol; perfluorinated organic compounds; silicones; etc. But those products generally give a temporary water-repellency as they are removed little by little during repeated washings and degreasings of fabrics on which they are applied; this disadvantage is even more apparent when the agents used have a structure not allowing them to react with fabric cellulose and/or when they are used for treating textile materials on which they cannot be bound chemically. Moreover when those compounds are deposited on fabrics in the form of aqueous dispersions, it is necessary to add emulsifying agents to improve wetting; however, those hydrophilic products decrease the effect obtained by waterproofing agents.

It is a prime object of the present invention to provide new products and a process for their application, which obviates the precited disadvantages, and this has now been accomplished. One aspect of the invention relates to organic compounds intended for waterproofing textiles. Another aspect relates to a process of applying those compounds, providing an excellent water-repellency to all the types of textile materials, such water-repellency having especially the advantage of permanency, that is the ability to resist to repeated washings and degreasings.

The new waterproofing agents according to the invention are organic compounds having the general formula:



in which R is a tolylene or hexamethylene radical, A and B, identical or different, may be groups  $NHR_1$  or  $NHR_2$ ,  $N(R_1)_2$  or  $N(R_2)_2$ ,  $OR_1$  or  $OR_2$ ,  $R_1$  or  $R_2$ , in which  $R_1$  and  $R_2$ , identical or different, are aliphatic hydrocarbon radicals of the formula  $C_nH_{2n+1}$ ,  $n$  being an integer comprised between 12 and 22.

Those compounds exist under normal conditions in the form of white crystalline solids, quite soluble in hot, usual

2

organic solvents such as aromatic hydrocarbons, as benzene, toluene, or chlorinated aromatic hydrocarbons such as mono-, di-, trichlorobenzenes. In cold solvents their solubility is variable according to the particular compounds; however, even when cold their solubility is generally sufficient for the contemplated application, in solvents such as 1,2-dichloro, or 1,3,5-trichloro-benzene, or nitrobenzene.

Those compounds may be obtained by means of any classical techniques in the field of the contemplated products. As an example, they may be formed from tolylene- or hexamethylene-diisocyanate. Tolylene diisocyanate may be constituted by a mixture of isomers and especially be the commercial product containing 20% isomer 2,6 and 80% isomer 2,4 known under the name of Desmodur T80 (registered trademark). About symmetric derivatives, that is derivatives of which the radicals A and B are identical, bis-ureas may be prepared by reaction of the convenient isocyanate and amine, in an organic solvent which is inert under reaction conditions, specially a chlorobenzene or acetone. Biscarbamates are obtained by heating of convenient isocyanate and alcohol in an inert solvent in the presence of a tertiary amine as a catalyst. Or bis-amides may be prepared by reacting hexamethylene or tolylene-diisocyanate with an aliphatic acid, in the presence of a catalyst which may be a tertiary amine.

The asymmetric derivatives may have either different hydrocarbon radicals  $R_1$  and  $R_2$  or different functional groups—urea—carbamate—amide, or those two differences at the same time. In the first case the compounds are obtained by means of the precited methods in reacting simultaneously on isocyanate the two types of necessary reagents; in the other cases a two-stage process is necessary.

Examples of the present compounds are hexamethylene-bis-(3-octadecylurea); hexamethylene-bis-octadecanamide; hexamethylene-bis-(O-tetradecyl carbamate); the 2,4 and 2,6 isomers, alone or in admixture, of tolylene-bis(3-dodecylurea), of tolylene-bis(3-tetradecylurea), of tolylene-bis(3-hexadecylurea), of tolylene-bis(3-octadecylurea), of tolylene-bis(3-dioctadecylurea), tolylene-bis(O-tetradecyl carbamate), tolylene-bis(O-octadecyl carbamate), of tolylene-bis(O-eicosyl carbamate), of tolylene-bis-hexadecanamide, of tolylene-bis-octadecanamide, of tolylene (3-dodecylurea-3'-octadecylurea), of  $N[(3\text{-octadecylureido})\text{ tolylene}]$  octadecanamide, and of octadecyl  $N[(3\text{-octadecylureido})\text{ tolylene}]$  carbamate.

The process of applying such waterproofing agents to textiles, which is also an object of the present invention, consists essentially of impregnating textiles with organic solutions of such agents, then of cross-linking the agents by means of polyisocyanates. Practically the process is generally carried out by providing organic solutions of the waterproofing agent, to which is added the polyisocyanate used for further cross-linking, and possibly a catalyst of known type which accelerates this reaction, then in applying this solution on the fabric by any classical method such as spraying or padding, and then, after solvent removing, in submitting the fabric to a thermal treatment in order to obtain cross-linking.

The concentration of the waterproofing agent in the organic solution may vary within large limits. It is, however, advantageous to use between 20 and 100 gm. per liter of solution. The solvents which may be used are the ones which have been quoted hereinabove as suitable for dissolving the compounds of Formula I in the hot or cold. At the hereinabove given concentrations the obtained solutions are slightly viscous and have a translucent appearance.

As isocyanates for cross-linking the waterproofing agents, all the types of known di- and polyisocyanates may be used, and for example hexamethylene-diisocya-

cate or its reaction product with water having the commercial name of Desmodur N (registered trademark); tolylene-diisocyanate and especially the mixture of precited isomers, known under the name of Desmodur T80; diphenyl-methane diisocyanate; the mixture of diphenyl-methane diisocyanate and of its higher homologs having the commercial name of Desmodur VL (registered trademark); a polyisocyanate having an isocyanurate structure, such as Desmodur IL (registered trademark); a tri-isocyanate resulting from condensing trimethylol propane and tolylene diisocyanate, such as Desmodur L (registered trademark), etc. The quantity of isocyanate to be used must be at least equal to that theoretically necessary to cross-link the waterproofing agent. However, it is preferred to use an excess of isocyanate, for example, 50 to 150% excess, i.e. 150-250% based on 100% agent.

As stated above, it is possible to add to the solution catalysts of known type, which accelerate the reaction between waterproofing agent and polyisocyanate. The convenient accelerating agents are, for example, tertiary amines such as methyl diethyl amine, triethyl amine, N-methyl morpholine, organo-metallic compounds, such as tetramethyl tin, dibutyl tin dilaurate, metal salts of organic acids such as zinc octanoate, cobalt naphthenate, etc.

It is interesting to note that the mixtures prepared in this way, containing the derivative of Formula I in solution, polyisocyanate and optionally, reaction accelerating agent, are stable in the cold and may be kept as such for several days. They are applied on fabrics at room temperature or at a higher temperature, for example at 50-80° C.

As stated above, the textile material is impregnated according to classical technique such as spraying or padding, followed by squeezing. The quantity of impregnating solution is adjusted, taking into account its concentration, in order to obtain the desired proportion of dry extract (calculated on the basis of waterproofing agent + polyisocyanate) on fabric. This proportion is favorably comprised between 0.5 and 5%, preferably 1 to 3% with regard to the weight of the treated textile.

After solvent removing cross-linking is induced in situ by submitting the fabric to a thermal treatment. The applied temperatures are in a range which is not harmful for treated textiles. Indeed it is operated at temperatures, which, with regard to the used polyisocyanate, vary in a general way between 100 and 150° C. The reaction is quick enough; thus, after a treatment time of 3 to 4 minutes, it is possible to have a sufficient cross-linking. Generally, a complete reaction is obtained in submitting fabric to precited temperatures during a time which does not exceed 15 min. and which is, the most usually, from 5 to 7 minutes.

The new waterproofing agents and the application process according to the invention, may be used for all the types of textiles, constituted either by natural fibers such as cotton, linen, wool or blends, or artificial fibers such as viscose, rayon, cellulose acetates, or synthetic fibers such as polyacrylic fibers, polyesters, polyamides, or still by their mixtures as for example associations polyester-cotton, polyester-viscose, etc. They are especially interesting for synthetic textiles such as polyamides, which, it is known, are the most difficult to hydrofuge. The obtained waterproofing is at the beginning generally superior than the one brought about by known products and it resists conveniently to washings and/or degreasings much better than the known materials.

The examples hereinafter, given in a non-limitative way, further illustrate the object of the invention. Examples 1 to 5 describe the preparation of waterproofing agents. The following examples relate to tests of waterproofing various textiles.

#### EXAMPLE 1

For this test a device has been used which was constituted by a reactor provided with a stirrer, a thermo-

couple, a system for introducing isocyanate and surrounded by a cooler.

300 kg. of monochlorobenzene and 50 kg. of octadecylamine were fed to the reactor. The mixture was brought to 80° C.; then there was introduced during 1 hour under strong stirring, 16 kg. of Desmodur T80 (tolylene-diisocyanate with 80% of isomer 2,4 and 20% of isomer 2,6) maintaining temperature between 85 and 95° C. After cooling, the reaction mixture was filtered, then the isolated white solid was washed with acetone. After drying there was recovered 62.7 kg. of a product melting at 175° C.

The product has been identified as being a mixture of the 2,4 and 2,6 isomers of tolylene-bis (3-octadecylurea).

Results of elemental analysis.—Calculated (percent): C, 75.78; H, 11.87; N, 7.85. Found (percent): C, 75.70; H, 11.86; N, 7.77.

In operating under the same conditions as hereinabove, but in replacing Desmodur T by hexamethylene-diisocyanate, there was obtained hexamethylene-bis (3-octadecyl-urea) melting at 175-176° C.

#### EXAMPLE 2

In a device identical to the one of Example 1, there was loaded 160 kg. of acetone and 80 kg. of dioctadecylamine, at room temperature. Then there was introduced in 45 min. under strong stirring 13.4 kg. of Desmodur T80 in solution in 50 kg. of acetone, maintaining the temperature near 30° C. After the end of addition, the reaction mixture was heated under reflux for 1 hour. After cooling, the formed white crystalline solid was isolated by filtration; after air drying, it weighed 80 kg.

This product, the melting point of which is 53-55° C., has been identified as being a mixture of the 2,4 and 2,6 isomers of tolylene-bis (3-dioctadecylurea)-(nitrogen content: calculated 4.60; found 4.65).

#### EXAMPLE 3

In a device of the same type as in Example 1, there was introduced 1 kg. of trichlorethylene, 320 g. of 1-octadecanol and 1 g. of triethylamine, to which 110 g. of Desmodur T80 was added slowly. After cooling at 20° C. the reaction mixture was filtered and the isolated white solid was washed with acetone; this solid had a weight of 330 g. and has been identified as being a mixture of the 2,4 and 2,6 isomers of tolylene-bis (O-octadecyl carbamate). Its melting point is 90-92° C. (nitrogen content: calculated 3.92; found 4.03).

#### EXAMPLE 4

To a mixture of 1 kg. of octadecanoic acid and 5 gm. of triethylamine, heated to 170-180° C., was added 306 g. of Desmodur T80, under stirring. After the addition the mixture was maintained at 170-180° C. during 2 hr. 30 min. Then it was cooled to 100° C., cast, and thereafter ground. There was recovered 1.140 kg. of a white solid identified as being a mixture of 2,4 and 2,6 tolylene (bis-octadecanamide); after crystallization from dimethylformamide, this product melts at 133-135° C. (nitrogen content: calculated 4.27; found 4.20).

#### EXAMPLE 5

Octadecyl N-[(3-octadecyl-ureido) tolylene] carbamate was prepared in a 2 stage process by reacting first tolylene-diisocyanate with 1-octadecanol (molar ratio 1/1) in acetone, then introducing the necessary quantity of octadecylamine (1 mole per isocyanate mole), and at last filtering the reaction mixture for isolating the formed white precipitate. Then the product was washed with acetone and dried.

#### EXAMPLE 6

A solution of 50 g./l. of tolylene-bis (3-octadecylurea) from Example 1 was prepared in o-dichlorobenzene, by introducing under stirring the bis-urea into the solvent previously heated to 80° C. Then after cooling to 20° C.,

two formulations were made from this solution by adding:

| In the first case:       | Gr./l. |
|--------------------------|--------|
| Desmodur T80             | 25     |
| Zn octanoate             | 0.2    |
| In the second case:      |        |
| Desmodur VL <sup>1</sup> | 30     |
| Zn octanoate             | 0.2    |

<sup>1</sup> Mixture of primarily diphenyl methane diisocyanate and of its higher homologs (considered as pure diphenylmethane diisocyanate in the calculation for the test).

Then 2 pieces of polyester/cotton fabric were padded at room temperature, using the two formulations (1 piece per formulation) in order to have a deposit of about 2.0% of dry material on the fabric. They were dried at 60° C. and submitted to a thermal treatment of 5 minutes at 130° C. Then half of each fabric respectively was washed or degreased several times, and applied to them after the first and fifth operations was the "Schmerber test," well known in textile industry (standard Afnor G07-057). This test consists of measuring the maximal pressure of mm. water which may be borne by fabric before passage therethrough. (The test was also applied after treatment, before washing or degreasing.)

Washings were made by treatment at 60° C. during 30 minutes with an aqueous solution of 5 g./l. of soap and 2 g./l. of sodium carbonate (according to standard ISO3). Degreasings were achieved by means of perchlor-ethylene at 20° C., during 30 minutes.

The obtained results are given in the Table 1 herein-after:

per liter of o-dichlorobenzene was padded at 50° C., then dried at 60° C. Then the fabric was submitted to a temperature of 130° C. during 5 mintues. The deposit of dry material on the fabric was 3.0%.

In a comparative way, two samples of fabric identical to the previous one were treated in the same conditions as above, but using this time, instead of the products of the invention, known waterproofing agents applied according to their own techniques, that is:

10 Formula A: 100 gr./l. of paraffinic wax added with metallic salts, and applied as an aqueous emulsion  
Formula B: 120 gr./l. of stearylated melamine/formol resin applied as an aqueous emulsion brought to pH 4.5 by addition of acetic acid.

15 Then those different samples were submitted to washings, degreasings and to Schmerber test, as described in the previous examples. Moreover, another test, also classical in textile industry, was made on those fabrics, with the help of the apparatus called "Spray Tester" (see Afnor Standard G07-056 and ASTM Standard D583-63). This test measures the wettability of fabrics and the results are expressed according to the following scale:

20 1—Complete wetting of the hole watered surface  
2—Wetting of more than the half of watered surface  
3—Wetting of the watered surface, only on small separated zones  
4—No wetting, only small droplets adhere to the watered surface  
25 5—No wetting and no droplet on the watered surface.

TABLE 1.—RESULTS OF SCHMERBER TEST  
(mm. water)

|                    | After treatment | After first washing | After first degreasing | After 5th washing | After 5th degreasing |
|--------------------|-----------------|---------------------|------------------------|-------------------|----------------------|
| First formulation  | 180             | 180                 | 190                    | 145               | 185                  |
| Second formulation | 180             | 170                 | 195                    | 140               | 180                  |

### EXAMPLE 7

Cotton fabrics were treated in the same conditions and with the same formulations as in Example 6. Then they were submitted to the same test after washings and degreasings, as explained previously. The results are reproduced in the Table 2 hereinafter.

TABLE 2.—RESULTS OF SCHMERBER TEST  
(mm. water)

|                    | After treatment | After first washing | After first degreasing | After 5th washing | After 5th degreasing |
|--------------------|-----------------|---------------------|------------------------|-------------------|----------------------|
| First formulation  | 330             | 200                 | 200                    | 200               | 200                  |
| Second formulation | 210             | 190                 | 240                    | 210               | 220                  |

### EXAMPLE 8

A sample of polyamide 6-6 taffeta in a solution containing 50 g. of tolylene-bis (3-octadecylurea) of Example 1, 39 gr. of Desmodur VL and 0.2 gr. of zinc octanoate,

The obtained values are given in Table 3 hereinafter. The numbers correspond to the average of 4 measures achieved in 4 different points of the samples.

45 As it may be seen, the waterproofing degree given to fabrics by the techniques according to the invention, and valued according to Schmerber test is still higher, after 5

washings or degreasings, than the one initially brought by the techniques of prior art. Wettability numbers are also quite satisfactory while the results become quickly bad with Formulae A and B.

TABLE 3

|                            | Fabric treated             |              |                |              |                |
|----------------------------|----------------------------|--------------|----------------|--------------|----------------|
|                            | According to the invention |              | With Formula A |              | With Formula B |
|                            | Schmerber                  | Spray-tester | Schmerber      | Spray-tester | Schmerber      |
| Measurement results after— |                            |              |                |              |                |
| Treatment                  | 225                        | 5            | 75             | 5            | 82             |
| First washing              | 180                        | 4            | 75             | 3            | 75             |
| Second washing             | 160                        | 4            | 80             | 2            | 57             |
| Third washing              | 152                        | 3            | 67             | 2            | 60             |
| Forth washing              | 108                        | 3            | 67             | 2            | 31             |
| Fifth washing              | 104                        | 3            | 65             | 2            | 35             |
| First degreasing           | 137                        | 4            | 50             | 2            | 57             |
| Second degreasing          | 132                        | 4            | 38             | 1            | 36             |
| Third degreasing           | 137                        | 4            | 50             | 1            | 50             |
| Fourth degreasing          | 120                        | 4            | 50             | 1            | 24             |
| Fifth degreasing           | 106                        | 3            | 34             | 1            | 22             |

## EXAMPLE 9

There were prepared solutions at 50 gr./l. in orthodichlorobenzene, of every one of the compounds of Examples 2 through 5, by dissolution of said compounds in the solvent, under stirring, at room temperature. Then from these solutions two series of formulations were made, by adding:

For the first series:

|                    | G./l. |
|--------------------|-------|
| Desmodur T80       | 25    |
| Cobalt naphthenate | 0.2   |

For the second series:

|                    | G./l. |
|--------------------|-------|
| Desmodur VL        | 39    |
| Cobalt naphthenate | 0.2   |

These 8 compositions were used to pad samples of polyamide 6-6 to obtain a deposit of 2 to 3% of dry material on the fabric. Those fabrics were dried at 100° C. and a thermal treatment of 5 minutes was applied to them at 130° C.

The different samples were submitted to washings, de-greasings, Schmerber test and spray-tester as described in the previous examples.

The obtained results are shown in the Table 4 herein-after.

TABLE 4

| Formulation (series) | Fabric treated with the product of Example |     |      |     |      |     |      |     |      |     |      |     |      |     |  |  |
|----------------------|--------------------------------------------|-----|------|-----|------|-----|------|-----|------|-----|------|-----|------|-----|--|--|
|                      | 2                                          |     |      |     | 3    |     |      |     | 4    |     |      |     | 5    |     |  |  |
|                      | 1st                                        | 2d  | 1st  | 2d  | 1st  | 2d  | 1st  | 2d  | 1st  | 2d  | 1st  | 2d  | 1st  | 2d  |  |  |
| Tests                | Sch.                                       | Sp. | Sch. | Sp. | Sch. | Sp. | Sch. | Sp. | Sch. | Sp. | Sch. | Sp. | Sch. | Sp. |  |  |
| Results after—       |                                            |     |      |     |      |     |      |     |      |     |      |     |      |     |  |  |
| Treatment            | 125                                        | 4   | 120  | 5   | 140  | 5   | 130  | 5   | 140  | 5   | 125  | 5   | 105  | 5   |  |  |
| 5th washing          | 115                                        | 4   | 120  | 4   | 70   | 3   | 130  | 3   | 70   | 3   | 70   | 4   | 80   | 3   |  |  |
| 5th degreasing       | 90                                         | 3   | 105  | 3   | 80   | 3   | 80   | 4   | 90   | 4   | 80   | 3   | 75   | 3   |  |  |
|                      |                                            |     |      |     |      |     |      |     |      |     |      |     |      |     |  |  |

NOTE.—Schmerber Test (Sch.)—results given in mm. water; "Spray-tester" (Sp.).

The values reproduced above show that the waterproofing degree of polyamide fabrics is maintained at a satisfactory level, even after 5 washings or degreasings.

What is claimed is:

1. A dried coating on a textile comprising:  
a compound having the formula:



wherein R is a tolylene or hexamethylene radical, A and B are selected from the group consisting of NHR<sub>1</sub>, NHR<sub>2</sub>, N(R<sub>1</sub>)<sub>2</sub>, N(R<sub>2</sub>)<sub>2</sub>, OR<sub>1</sub>, OR<sub>2</sub>, R<sub>1</sub> and R<sub>2</sub> in which R<sub>1</sub> and R<sub>2</sub> are selected from the group consisting of aliphatic hydrocarbon radicals of formula C<sub>n</sub>H<sub>2n+1</sub>, n being an integer between 12 and 22, inclusive;

5 said compound being cross-linked with a polyisocyanate in the presence of an accelerator.

2. A cross-linked waterproofing coating on a textile comprising:  
5 a compound having the formula



wherein R is a tolylene or hexamethylene radical, A and B are selected from the group consisting of NHR<sub>1</sub>, NHR<sub>2</sub>, N(R<sub>1</sub>)<sub>2</sub>, N(R<sub>2</sub>)<sub>2</sub>, OR<sub>1</sub> OR<sub>2</sub> R<sub>1</sub> and R<sub>2</sub> in which R<sub>1</sub> and R<sub>2</sub> are selected from the group consisting of aliphatic hydrocarbon radicals of formula C<sub>n</sub>H<sub>2n+1</sub>, n being an integer between 12 and 22, inclusive;

said compound being condensed with a polyisocyanate.

## References Cited

## UNITED STATES PATENTS

|    |           |        |                                |
|----|-----------|--------|--------------------------------|
| 40 | 2,314,968 | 3/1943 | Berstian et al. — 117—139.5 A  |
|    | 2,343,920 | 3/1944 | Maxwell — 117—139.5 CQ         |
|    | 2,446,864 | 8/1948 | Abrams — 117—143 A             |
|    | 2,555,745 | 6/1951 | Hopkins et al. — 117—138.8 U A |
| 45 | 3,119,865 | 1/1964 | Weakley et al. — 260—553 A     |
|    | 3,384,606 | 5/1968 | Dieterich et al. — 117—161 KP  |
|    | 3,392,148 | 7/1968 | Zech et al. — 117—161 KP       |

## FOREIGN PATENTS

|         |        |                        |
|---------|--------|------------------------|
| 118,839 | 8/1944 | Australia — 117—DIG. 7 |
|---------|--------|------------------------|

50 WILLIAM D. MARTIN, Primary Examiner

T. G. DAVIS, Assistant Examiner

## U.S. CL. X.R.

117—138.8 F, 138.8 N, 138.8 UA, 141, 143 R, 144

UNITED STATES PATENT OFFICE  
CERTIFICATE OF CORRECTION

Patent No. 3,788,884 Dated January 29, 1974

Inventor(s) ANDRE BERNARD et al

It is certified that error appears in the above-identified patent and that said Letters Patent are hereby corrected as shown below:

Column 5, line 20, "Afnor" should read --AFNOR--

Column 5, Table 2, "330" should read --220--

Column 6, line 20, "Afnor" should read --AFNOR--

Column 6, line 24, "hole" should read --whole--

Signed and sealed this 16th day of July 1974.

(SEAL)

Attest:

MC COY M. GIBSON, JR.  
Attesting Officer

C. MARSHALL DANN  
Commissioner of Patents